

**United States Patent**

[11] 3,590,996

[72] Inventor **Guy H. Harris**  
Concord, Calif.  
[21] Appl. No. 796,159  
[22] Filed Feb. 3, 1969  
[45] Patented July 6, 1971  
[73] Assignee **The Dow Chemical Company**  
Midland, Mich.

3,290,351 12/1966 McKay ..... 260/455

## FOREIGN PATENTS

|           |         |                     |         |
|-----------|---------|---------------------|---------|
| 750,568   | 6/1956  | Great Britain ..... | 260/455 |
| 1,179,312 | 12/1958 | France .....        | 260/455 |

Primary Examiner—Tim R. Miles

*Assistant Examiner—Robert Halper*

Attorneys—Griswold and Burdick

Howard and Bardick and Bruce M. Kanuch

[54] **FLOTATION OF SULFIDE ORES**  
**10 Claims, No Drawings**

|      |                      |                                  |
|------|----------------------|----------------------------------|
| [52] | U.S. Cl.....         | 209/166,<br>200/455              |
| [51] | Int. Cl.....         | B03d 1/02,<br>C07c 153/07        |
| [50] | Field of Search..... | 209/106,<br>167; 252/61; 260/455 |

[56] References Cited

UNITED STATES PATENTS

| NAME      |         | PATENT        |           |
|-----------|---------|---------------|-----------|
| 1,640,218 | 8/1927  | Sayre.....    | 209/166   |
| 1,674,166 | 6/1928  | Douglass..... | 209/166   |
| 2,691,635 | 10/1954 | Harris.....   | 209/166 X |
| 2,835,625 | 5/1958  | Lo.....       | 260/455 X |
| 3,012,053 | 12/1961 | Lesslie.....  | 260/455   |
| 3,224,863 | 12/1965 | D'Amico.....  | 260/455 X |

**ABSTRACT:** An improvement in the concentration of ores by flotation which comprises subjecting a sulfide ore in the form of a pulp to a flotation process in the presence of an effective quantity of a flotation collector corresponding to the formula



wherein R and R<sub>2</sub> are hydrocarbyl groups and R<sub>1</sub> represents an alkylene or heteroalkylene group. Certain of the indicated compounds provide for enhanced recovery and/or selectivity of sulfide minerals of Cu, Zn, Mo, Co, Ni, Pb and As over iron sulfide. The compounds are also useful as fungicides and herbicides.

## FLOATATION OF SULFIDE ORES

## BACKGROUND

Flotation is a process of treating a mixture of finely divided mineral solids, e.g., a pulverulent ore suspended in a liquid whereby a portion of such solids are separated from other finely divided mineral solids, e.g., clays and other like materials present in the ore, by introducing a gas (or providing a gas in situ) in the liquid to produce a frothy mass containing certain of the solids on the top of the liquid, and leaving suspended (unfrothed) other solid components of the ore. Flotation is based on the principle that introducing a gas into a liquid containing solid particles of different materials suspended therein causes adherence of some gas to certain suspended solids and not to others and makes the particles having the gas thus adhered thereto lighter than the liquid. Accordingly, they rise to the top of the liquid to form a froth.

Various flotation agents have been admixed with the suspension to improve the frothing process. Such added agents are classed according to the function to be performed: collectors, e.g., high carbon chain compounds such as collectors for sulfide minerals including xanthates, thionocarbonates, and the like; frothers which impart the property of forming a stable froth, e.g., natural oils such as pine oil and eucalyptus oil; modifiers such as activators to induce flotation in the presence of a collector, e.g., copper sulfate; depressants, e.g., sodium cyanide, which tend to prevent a collector from functioning as such on a mineral which it is desired to retain in the liquid, and thereby discourage a substance from being carried up and forming a part of the froth; pH regulators to produce optimum metallurgical results, e.g., lime, soda ash and the like.

It is of importance to bear in mind that additives of the above type are selected for use according to the nature of the ore, the mineral sought to be recovered, and the other additaments which are to be used in combination therewith.

An understanding of the phenomena which makes flotation a particularly valuable industrial operation is not essential to the practice of the present invention. They appear, however, to be largely associated with selective affinity of the surface of particulated solids, suspended in a liquid containing entrapped gas, for the liquid on one hand, the gas on the other.

The flotation principle is applied in a number of mineral separation processes among which is the selective separation of such minerals as sulfide copper minerals, sulfide zinc minerals, sulfide molybdenum minerals and others from sulfide iron minerals. The present invention concerns a novel class of compounds. These compounds can be employed as collection agents in a flotation process. With some of these compounds better recoveries are realized and with others, improved selectivity is achieved. Certain of these compounds produce improvement in both aspects.

## SUMMARY

The present invention concerns novel compounds corresponding to the formula



wherein R represents H, a hydrocarbyl group, or a heterohydrocarbyl group, wherein said groups can be substituted with up to two functional groups and contain from 1 to 10 carbon atoms; R<sub>1</sub> represents an alkylene or heteroalkylene group having a heteroatom substituted in the carbon chain, and R<sub>2</sub> represents a hydrocarbyl or heterohydrocarbyl group, except for aryl, wherein either of said groups can be substituted except in the alpha position with up to two functional groups. The novel compounds can be prepared by the reaction of an amino alcohol with a xanthate ester and contacting the product produced with an acyl halide. The novel compounds can be employed to improved the flotation

process of separating sulfide minerals from ores by employing an effective quantity of at least one of the novel compounds set forth herein in the flotation process. The novel compounds are also useful as fungicides and herbicides.

## PREFERRED EMBODIMENTS

The novel compounds of the present invention correspond to the formula



wherein R represents H, a hydrocarbyl group selected from the group consisting of alkyl or alkenyl containing up to 10 carbon atoms, alkaryl, aryl, aralkyl, cycloalkyl, cycloalkenyl, aralkenyl or acylalkyl groups, wherein the acyclic carbon chain portions preferably contain up to 3 carbon atoms and the cyclic group contains from 5 to 10 carbon atoms and a heterohydrocarbyl radical selected from the group consisting of alkoxy, alkenyloxy, alkoxy carbonyl, alkoxy carbonylalkyl, aryloxy, arylalkoxy, alkylthio and arylthio groups, wherein said heterohydrocarbyl groups can contain up to two identical or different functional groups preferably selected from the group consisting of halo, alkoxy, cyano, and di-loweralkylamino groups; R<sub>1</sub> represents an alkylene or heteroalkylene group containing up to 8 carbon atoms and wherein the hetero atom is substituted in the carbon chain and is preferably selected from the group consisting of



wherein X is a hydrocarbyl or heterohydrocarbyl group and not H; preferably X is a lower alkyl group containing up to 5 carbon atoms; and R<sub>2</sub> represents a hydrocarbyl group selected from the group consisting of an alkyl or alkenyl group, preferably containing up to 8 carbon atoms, an aralkyl group, preferably containing from 1 to 3 carbon atoms, in the alkyl portion, and an alicyclic or cycloalkenyl group, preferably containing from 3 to 8 carbon atoms, wherein said hydrocarbyl groups can be substituted, except in the alpha position, with up to two identical or different functional groups preferably selected from the group consisting of alkoxy, halo, cyano, acetonyl and dilower alkylamino groups. R, R<sub>1</sub>, and R<sub>2</sub> are further characterized in that the total number of carbon atoms in said groups preferably ranges from about 4 to about 25.

The novel compounds as defined herein can be prepared, for example, by reacting an aminoalcohol with a xanthate ester to prepare a hydroxy-thionourethane and then acylating the HO-R<sub>1</sub>-moiety with an acyl halide, anhydride, or ketene. The reactions can be represented as follows:



The novel compounds as defined herein have a special utility as flotation collectors and can be employed in standard flotation processes to concentrate copper sulfide and other like minerals from sulfide ores in preference to iron sulfides. In a flotation process a pulp is first prepared by wet grinding a sulfide containing ore to a suitable size with or without a pH modifier. A suitable frothing agent is then added, e.g., pine oil, cresylic acid, polyalkoxyparaffin and the like. An effective quantity of a flotation collector compound as defined herein is

then added, usually ranging from about 0.01 lbs. to about 0.25 lbs. per ton of pulp, and the pulp is usually agitated and aerated. Sulfide minerals, e.g., copper, nickel, zinc, molybdenum sulfides, and other like sulfide minerals collect as a froth which is readily overflowed or skimmed off from the residual gangue and other undesired materials and the metal values therein recovered.

The following Examples will facilitate a more complete understanding of the present invention but they are not meant to limit the scope of the invention to the specific embodiments incorporated therein.

#### Example 1

A novel compound corresponding to the formula



was prepared in the following manner.

To 30 grams (0.2 moles) of methyl isopropyl xanthate was added 12.2 grams (0.2 moles) of 2-aminoethanol. The mixture became hot and there was a vigorous evolution of methyl mercaptan. After an hour of heating on the steam bath, the residual methyl mercaptan was removed by applying a vacuum. The structure of the product, confirmed by infrared and NMR analyses, corresponded to the formula



The product was a viscous liquid. A sample of this product was distilled under vacuum and had a boiling point of 120-122° C. at 0.7 mm. Hg.

A solution of 16.3 grams of the product prepared above, 10.2 grams of acetic anhydride, and 8.1 ml. of pyridine in 100 ml. of absolute diethyl ether was let stand for a day. More ether was added and then the mixture was washed twice with water, dilute HCl, and finally with saturated aqueous NaHCO<sub>3</sub>. After drying over MgSO<sub>4</sub> and removing the solid by filtration, the solvent was stripped off by heating to 75° C. under a reduced pressure of 20 mm. The yield was 16.9 grams (76.5 percent yield) of the novel compound designated above. The structure of the new compound was identified by infrared analysis. A sample of the compound was distilled under a reduced pressure and was found to have a boiling point of 109-112° C. at 0.1 mm. Hg.

#### Example 2

A new compound within the scope of the invention defined herein and corresponding to the formula



was prepared in the following manner: A solution of 16.3 grams of isopropyl 2-hydroxyethylthionocarbamate in 25 ml. of 50 percent diketene/acetone was let stand for a week. The oil obtained on addition of 100 ml. of water was taken up in ether. This extract was dried over MgSO<sub>4</sub>. The solid was later removed by filtration and the ether removed by distillation, the last traces with a vacuum. The structure as set forth above was confirmed by infrared and NMR analyses. The yield was 89 percent. The calculated and actual elemental analysis for the product corresponding to the formula set forth above is

| Percent            |      |      |
|--------------------|------|------|
| C                  | H    | N    |
| Calculated... 48.6 | 6.88 | 5.67 |
| Actual..... 48.5   | 6.7  | 5.6  |

#### Example 3

Another novel compound within the scope of the present invention is prepared in the following manner. The reaction is set forth as:



The compound is prepared as follows.

To 15 grams (0.1 g. mole) of methyl isopropyl xanthate is added 14.5 g. (0.1 g. mole) of 2-aminoethyl pivalate and the mixture warmed. When methyl mercaptan evolution ceases, the last traces are removed under vacuum. The residual oil is induced to crystallize and the resulting solid—the new compound—is found to melt at 48-49° C.

#### Example 4

A new compound corresponding to the formula



was prepared in the following manner.

A solution of 16.3 grams of isopropyl 2-hydroxyethylthionocarbamate (0.1 mole), 7.9 gms. of pyridine (0.1 mole) in 100 ml. of ether, was cooled and stirred. 13.6 grams (0.1 mole) of ethyl oxalyl chloride was added with cooling and stirring and when this was complete, the solution was stirred for one hour. The ether solution was dried with Na<sub>2</sub>SO<sub>4</sub>, filtered and stripped of ether by heating under a vacuum. The product yield was 81 percent. The product was analyzed by both infrared and NMR analysis. The actual and calculated elemental analysis for the compound having the formula set forth above are:

| Percent             |      |      |
|---------------------|------|------|
| C                   | H    | N    |
| Calculated... 45.61 | 6.51 | 5.32 |
| Actual..... 44.0    | 6.50 | 5.80 |

#### Example 5

A new compound within the scope of the present invention was prepared corresponding to the formula



A starting material compound corresponding to the formula



was prepared as follows: To 18.1 grams of 2-(2-hydroxyethyl)-thioethylamine was added 22.5 grams of methyl isopropyl xanthate. The mixture was heated in a hot water bath to drive off most of the evolved CH<sub>3</sub>SH gas. The mixture was then heated to 65° C. under a reduced pressure of 20 mm. to remove the last traces of CH<sub>3</sub>SH. The yield was nearly quantitative. The structure of this starting material was by infrared and NMR analysis. To 17.9 grams of the so-prepared starting material in 35 ml. of ether and 8.9 ml. of pyridine was added 9.0 grams of acetic anhydride. After 20 hours, additional ether and a small quantity of methanol was added to convert the unreacted acetic anhydride present to methyl

acetate. The reaction mixture was then treated with a dilute hydrochloric acid solution to remove the pyridine and then washed with aqueous  $\text{NaHCO}_3$  to remove the acids. The product mixture was then dried over  $\text{MgSO}_4$ , filtered and the remaining ether and the methyl acetate were removed under reduced pressure of 4 mm. by heating to 70° C. 19.7 grams or about a 93 percent yield of the product was obtained. The structure of the novel compound corresponding to that set forth above was confirmed by infrared and NMR analysis. Elemental analysis gave C-45.2 percent, H-6.8 percent and N-5.6 percent. Calculated analysis for a compound corresponding to the above structure is C-45.3 percent, H-7.2 percent and N-5.3 percent.

## Example 6

Other species of compounds within the scope of the present invention were prepared according to one of the procedures set forth in Examples 1-4. The starting materials consisted of a compound corresponding to the formula



and an acylating agent which provided the



moiety of the novel compounds.  $\text{R}_1$ ,  $\text{R}_2$ , the acylating agent, the empirical formula of the prepared compound, and the actual and calculated analysis for each compound are set forth in the following Table I. The method of preparation is listed in the method of preparation column and the number corresponds to one of the Examples 1-4. All the compounds were found to possess collector activity when employed in the flotation separation of sulfide containing ores.

20

25

30

35

## Example 7

Various species of flotation collector compounds within the scope of the present invention were employed in the recovery of copper and molybdenum from a sulfide ore obtained from South America employing the following procedure: The ore sample was ground for 5 minutes at 66 percent solids with no reagents. The pulp was then conditioned for 8 minutes with 0.12 lbs./ton of a specific flotation collector compound and 10 0.13 lbs./ton of a standard frother. During the conditioning period the pH was adjusted to a value of about 3.8. The pulp was then floated for seven minutes and the tailings assayed for copper and molybdenum. A standard flotation collector consisting of a thionocarbamate compound corresponding to the formula



TABLE I

| Compound empirical                               | Method of preparation | $\text{R}_1$                                                | $\text{R}_2$            | Acylating agent                                                                      | Analysis, percent |      |      |        |     |     |
|--------------------------------------------------|-----------------------|-------------------------------------------------------------|-------------------------|--------------------------------------------------------------------------------------|-------------------|------|------|--------|-----|-----|
|                                                  |                       |                                                             |                         |                                                                                      | Calculated        |      |      | Actual |     |     |
|                                                  |                       |                                                             |                         |                                                                                      | C                 | H    | N    | C      | H   | N   |
| $\text{C}_8\text{H}_{12}\text{N O}_3\text{S}$    |                       | 1 $-\text{CH}_2\text{CH}_2-$                                | $-\text{iPr}^a$         | $(\text{CH}_3\overset{\text{O}}{\underset{\text{C}}{\text{C}}})_2\text{O}$           | 46.81             | 7.37 | 6.82 | 46.4   | 7.3 | 6.8 |
| $\text{C}_{14}\text{H}_{16}\text{N O}_3\text{S}$ |                       | 1 $\overset{\text{CH}_3}{\text{CH}}-\text{CH}_2-$           | $-\text{iPr}$           | $(\phi\overset{\text{O}}{\underset{\text{C}}{\text{C}}})_2\text{O}^b$                | 59.76             | 6.80 | 4.98 | 59.5   | 6.9 | 5.4 |
| $\text{C}_9\text{H}_{17}\text{N O}_3\text{S}$    |                       | 1 $-\text{CH}_2-\overset{\text{C}_2\text{H}_5}{\text{CH}}-$ | $-\text{C}_2\text{H}_5$ | $(\text{CH}_3\overset{\text{O}}{\underset{\text{C}}{\text{C}}})_2\text{O}$           | 49.29             | 7.82 | 6.39 | 49.4   | 8.2 | 4.9 |
| $\text{C}_9\text{H}_{17}\text{N O}_3\text{S}$    |                       | 1 $-\text{CH}_2-\overset{\text{CH}_3}{\text{CH}}-$          | $-\text{iPr}$           | $(\text{CH}_3\overset{\text{O}}{\underset{\text{C}}{\text{C}}})_2\text{O}$           | 49.29             | 7.82 | 6.39 | 48.6   | 8.0 | 6.5 |
| $\text{C}_{12}\text{H}_{22}\text{N O}_4\text{S}$ |                       | 1 $-\text{C}_2\text{H}_4\text{O C}_2\text{H}_4-$            | $-\text{iPr}$           | $(\text{CH}_3)_2\text{CH}\overset{\text{O}}{\underset{\text{C}}{\text{C}}}-\text{O}$ | 55.14             | 8.87 | 5.36 | 51.4   | 9.8 | 5.3 |
| $\text{C}_9\text{H}_{17}\text{N O}_4\text{S}$    |                       | 4 $-\text{C}_2\text{H}_4-$                                  | $-\text{iPr}$           | $\text{C}_2\text{H}_5\overset{\text{O}}{\underset{\text{C}}{\text{C}}}-\text{Cl}$    | 45.94             | 7.28 | 5.95 | 45.7   | 7.3 | 6.4 |
| $\text{C}_9\text{H}_{17}\text{N O}_3\text{S}$    |                       | 1 $-\text{CH}_2\overset{\text{CH}_3}{\text{CH}}-$           | $-\text{iPr}$           | $(\text{CH}_3\overset{\text{O}}{\underset{\text{C}}{\text{C}}})_2\text{O}$           | 49.29             | 7.82 | 6.39 | 48.6   | 8.0 | 6.5 |
| $\text{C}_{10}\text{H}_{19}\text{N O}_4\text{S}$ |                       | 4 $-\text{CH}_2\overset{\text{CH}_3}{\text{CH}}-$           | $-\text{iPr}$           | $\text{C}_2\text{H}_5\overset{\text{O}}{\underset{\text{C}}{\text{C}}}-\text{Cl}$    | 48.17             | 7.68 | 5.62 | 47.3   | 7.9 | 6.9 |
| $\text{C}_{13}\text{H}_{17}\text{N O}_3\text{S}$ |                       | 4 $-\text{C}_2\text{H}_4-$                                  | $-\text{iPr}$           | $\phi\overset{\text{O}}{\underset{\text{C}}{\text{C}}}-\text{Cl}$                    | 58.40             | 6.41 | 5.24 | 58.6   | 6.4 | 7.1 |
| $\text{C}_{11}\text{H}_{21}\text{N O}_3\text{S}$ |                       | 1 $-\text{C}_5\text{H}_{12}-$                               | $-\text{C}_2\text{H}_5$ | $(\text{CH}_3\overset{\text{O}}{\underset{\text{C}}{\text{C}}})_2\text{O}$           | 53.41             | 8.56 | 5.66 | 53.2   | 8.6 | 6.2 |
| $\text{C}_{12}\text{H}_{17}\text{N O}_4\text{S}$ |                       | 4 $-\text{C}_2\text{H}_4-$                                  | $-\text{iPr}$           | $\phi\overset{\text{O}}{\underset{\text{C}}{\text{C}}}-\text{Cl}$                    | 55.10             | 6.05 | 4.94 | 56.7   | 8.9 | 5.2 |

<sup>a</sup>— $\text{CH}(\text{CH}_3)_2$ .

<sup>b</sup>  $\phi$  is 

was employed as a control. The specific collector compounds employed and results are set forth in the following Table II.

TABLE II

| Run Number | Collector compound | Lbs./ton added | Percent Cu in tail | Percent Cu recovered | Percent Mo recovered |
|------------|--------------------|----------------|--------------------|----------------------|----------------------|
| Control.   | Control            | 0.12           | 0.281              | 84.2                 | 64.4                 |
| 1.         |                    | 0.08           | 0.228              | 87.2                 | 68.9                 |
| 2.         |                    | 0.09           | 0.234              | 87.0                 |                      |
| 3.         |                    | 0.03           | 0.238              | 86.6                 |                      |

## Example 8

Various novel collectors within the scope of the present invention were tested on a copper sulfide ore from the Southwestern United States. The ore sample was ground for 4½ minutes at 59 percent solids with 2.0 lbs./ton of lime. The pulp was conditioned for 2 minutes with an amount of a specific collector and 0.16 lbs./ton of a standard frother at a pH of 10.5. The pulp was then floated for 8½ minutes and the tailings assayed for copper. The results obtained are set forth in the following Table III. The same control flotation collector was employed as in Example 7.

In this example a copper-molybdenum sulfide containing ore from Western United States was treated in a manner similar to that described in Examples 7 and 8.

A sample of ore was ground at 60 percent solids to 35 percent minus 200 mesh Tyler. To the pulp was added 0.9 lbs./ton lime, 0.08 lbs./ton diesel oil, 0.01 lbs./ton of a collector compound to be tested and 0.06 lbs./ton frother. The ore was floated for 8 minutes. Both the concentrate and tailings were filtered, dried and assayed for Mo and Cu. The same control collector compound was employed as in Examples 7 and 8.

TABLE III

| Run Number | Collector compound | Lbs. ton added | Percent Cu in tail | Percent Cu recovered |
|------------|--------------------|----------------|--------------------|----------------------|
| Control    | Control            | 0.008          | 0.295              | 63.6                 |
| Do         | do                 | 0.16           | 0.133              | 82.7                 |
| 1.         |                    | 0.008          | 0.324              | 60.1                 |
| 2.         |                    | 0.008          | 0.298              | 62.8                 |
| 3.         |                    | 0.008          | 0.184              | 65.3                 |
| 4.         |                    | 0.025          | 0.092              | 87.2                 |
| 5.         |                    | 0.025          | 0.103              | 86.6                 |
| 6.         |                    | 0.025          | 0.113              | 84.4                 |
| 7.         |                    | 0.025          | 0.133              | 82.3                 |
| 8.         |                    | 0.13           | 0.110              | 85.5                 |
| 9.         |                    | 0.13           | 0.112              | 85.1                 |
| 10.        |                    | 0.13           | 0.117              | 84.6                 |
| 11.        |                    | 0.13           | 0.118              | 84.5                 |

The results obtained are shown in the accompanying Table IV.

prepare the indicated novel compound.

TABLE IV

| Run Number | Collector Compounds                                                                                                                                            | Lbs./ton | Tail, percent |       | Recovery, percent |      |
|------------|----------------------------------------------------------------------------------------------------------------------------------------------------------------|----------|---------------|-------|-------------------|------|
|            |                                                                                                                                                                |          | Mo            | Cu    | Mo                | Cu   |
| Control    | Control...                                                                                                                                                     | 0.01     | 0.003         | 0.029 | 57.1              | 83.4 |
| 1..        | H S                                                                                                                                                            | 0.01     | 0.004         | 0.025 | 50.0              | 86.1 |
| 2..        | $\text{C}_2\text{H}_5\text{OOCOC}_2\text{H}_4\text{NCOCH}(\text{CH}_3)_2$<br> | 0.01     | 0.005         | 0.038 | 44.4              | 78.2 |

The xanthate starting materials employed herein in the preparation of the novel compounds, for example, as in Example 1, can be prepared in a manner well known in the art. For example, an alcohol corresponding to  $\text{R}_2\text{OH}$ , wherein  $\text{R}_2$  is the same as defined hereinbefore, can be reacted as the corresponding alkali metal alkoxide, with  $\text{CS}_2$  to prepare a product corresponding to the formula



wherein  $\text{M}$  is the alkali metal ion. The product can then be contacted with, for example, methyl chloride, to prepare the corresponding xanthate ester



Alcohols which may be employed include, for example, 35 cyclohexanol, cyclohexenol, allyl alcohol, cinnamyl alcohol, 2-bromo-allyl alcohol; 2,3,5-trimethyl-3-hexanol; 2,3,4-trimethyl-2-hexanol and the like.

Acyling agents which can be used in preparing the novel compounds of the present invention can be prepared by converting carboxylic acids to the corresponding acyl chloride by contacting said acids with thionyl chloride by processes well known in the art. Carboxylic acids which may be employed include, for example, cinnamic acid,  $\alpha$ -bromocaproic acid, pelargonic acid, methacrylic acid, 3-cyanophenylacetic acid, cyclohexylacetic acid, cyanoacetic acid, 2-phenoxybutanoic acid, methoxyacetic acid and the like.

Other acylating agents which can be employed to prepare the novel compounds include thiocloroformates such as



and alkenylchloroformates such as



and the like.

Other novel compounds may be prepared in a manner similar to that described in the foregoing examples. For example, a compound corresponding to the formula



can be prepared by reacting ethylenimine and pivalic acid to prepare a compound corresponding to the formula



and reacting this compound with methyl isopropyl xanthate to

Another compound corresponding to the formula



is prepared by reacting 17.0 grams of aniosoyl chloride with 16.3 grams of ethyl 2-hydroxyethylthionocarbamate to produce the indicated compound having a molecular weight of 283. Similarly, by employing 10.4 grams of crotonyl chloride, 15.4 grams of crotonic anhydride, 13.8 grams of 2-chlorocrotonyl chloride, or 15.0 grams of 3-carbomethoxypropionyl chloride instead of aniosoyl chloride, compounds corresponding to the following formula are prepared:



and



respectively.

Other compounds within the scope of the present invention may be prepared by a method as defined herein by choosing various starting materials.

Various modifications may be made in the present invention without departing from the spirit or scope thereof for it is understood that we are limited only as defined in the appended claims.

50 What I claim is:

1. In a process of concentrating sulfide ores by flotation in the presence of a flotation collector, the improvement which comprises:

55 a. subjecting the sulfide containing ore in the form of a pulp to flotation collector comprising a compound corresponding to the formula



wherein  $\text{R}$  represents  $\text{H}$ , a hydrocarbyl radical selected from the group consisting of alkyl or alkenyl containing up to 10 carbon atoms, aryl, alkaryl, aralkyl, cycloalkyl, cycloalkenyl, aralkenyl or acylalkyl groups wherein the acyclic carbon chain portion contains up to 3 carbon atoms and the cyclic groups contains from 5 to 10 carbon atoms, a heterohydrocarbyl selected from the group consisting of alkoxy, alkenyloxy, alkoxy carbonyl, alkoxy carbonylalkyl, aryloxy, alkylthio, arylthio, or oxyalkyl group;  $\text{R}_1$  represents a member selected from the group consisting of an alkylene or heteroalkylene group containing up to 8 carbon atoms wherein the hetero atom in the heteroalkylene group is selected from the group consisting of

$-\text{O}-$ ,  $-\text{S}-$ , and  $-\text{N}-$ ,

wherein X is a member selected from the group consisting of a hydrocarbyl or heterohydrocarbyl radical wherein the hetero atom is substituted in the carbon chain; and R<sub>2</sub> represents a hydrocarbyl selected from the group consisting of an alkyl or alkenyl group, containing up to 8 carbon atoms, an aralkyl, containing from 1 to 3 carbon atoms in the alkyl portion, and an alicyclic or cycloalkenyl group, containing from 3 to 8 carbon atoms, wherein R, R<sub>1</sub> and R<sub>2</sub> are further characterized in that the total number of carbon atoms in said groups range from about 4 to about 25.

2. The process as defined in claim 1 wherein R and R<sub>2</sub> contain up to two functional groups other than in the alpha position of R<sub>2</sub>, selected from the group consisting of halo, alkoxy, cyano, acetonyl, or di-loweralkylamino group.

3. The process as defined in claim 1 wherein X is a lower alkyl group containing up to 5 carbon atoms.

4. The process as defined in claim 1 wherein from about 0.01 to about 0.25 pound of compound per ton of sulfide ore pulp is employed.

5. The process defined in claim 1 wherein said compound consists of



6. The process defined in claim 1 wherein said compound consists of



7. The process as defined in claim 1 wherein said compound consists of



8. The process as defined in claim 1 wherein said compound consists of



9. The process as defined in claim 1 wherein said compound consists of



25 10. The process as defined in claim 1 wherein said compound consists of

